

## 1

3,133,885

**METHOD OF INHIBITING METAL CORROSION  
BY AMINE-STABILIZED UNSATURATED CHLORINATED  
HYDROCARBONS (USING SUBSTITUTED OXIRANES)**

Wilbur H. Petering and William A. Callahan, Detroit, Mich., assignors to Detrex Chemical Industries, Inc., Detroit, Mich., a corporation of Michigan  
No Drawing. Original application July 23, 1954, Ser. No. 445,474. Divided and this application May 5, 1960, Ser. No. 26,942

14 Claims. (Cl. 252—153)

This a divisional application of our co-pending U.S. application Serial No. 445,474, filed July 23, 1954, and now abandoned.

This invention relates to a method of inhibiting the tarring and corrosion of certain metals such as iron or copper in the liquid phase of hot, dry amine-stabilized, unsaturated chlorinated hydrocarbons. Among the unsaturated chlorinated hydrocarbons to which the method of the present invention is applicable are trichlorethylene and perchlorethylene.

It is conventional in the art to add stabilizers of various types to chlorinated hydrocarbons. Among the accepted stabilizers are the phenolic compounds, amines, and various azo compounds. However, the choice of such compounds is quite limited except in the case of a few of the higher boiling chlorinated hydrocarbons, since most of the stabilizers also have relatively high boiling points. A wide difference in boiling points between the solvent and the stabilizers is undesirable because of the difficulty of stabilizing the vapor phase, and it is therefore desirable to provide a combination of a solvent and stabilizers not having wide differences in boiling points. Moreover, the distillation of the solvent may otherwise result in a complete loss of the stabilizer either in production or in subsequent use.

The organic amine bases have enjoyed widespread use as stabilizers for unsaturated chlorinated hydrocarbons. Such bases, including aliphatic amines and basic cyclic compounds characterized by nitrogen in the ring such as pyridine and the like are disclosed in the patents to Dinley, numbers 2,096,735, 2,096,736 and 2,096,737. Under many conditions the volatile aliphatic amine and/or heterocyclic nitrogen bases disclosed in the Dinley patents are highly effective and desirable stabilizers for chlorinated hydrocarbons. However, these stabilizers, as disclosed by Dinley, must boil fairly close to the solvent stabilized to have any real utility.

In the manufacture of unsaturated chlorinated hydrocarbons such as trichlorethylene, for example, the recovery of a neutral, sweet, relatively pure product is almost impossible without the use of a stabilizer such as amines. The amine stabilizer should be present in the refining operation, as distinguished from adding amine to the refined product, and the amine should be volatile with the chlorinated hydrocarbon and therefore carry over from the refining operation into the refined product. Unless a neutral, sweet product is obtained when the solvent is refined, subsequent attempts to stabilize the solvent often prove futile, or at least extremely costly and time con-

## 2

suming. Thus, the amines are not only highly effective and desirable stabilizers, but their use in both the liquid and vapor in the last stages of manufacture is almost essential.

5 Yet, in spite of the effectiveness and desirability of the amines as stabilizers, there appears to be an undesirable reaction or set of reactions which take place when the amines are used as stabilizers in unsaturated chlorinated hydrocarbon solvents in the presence of certain metals such as iron or copper or their alloys. It has now been discovered that the lower boiling unsaturated chlorinated hydrocarbons, when stabilized with certain of the conventional organic amines, such amines having boiling points 10 not widely different from the boiling points of the chlorinated hydrocarbons, appear to enter into a complex reaction when exposed to these metals, with resulting tarring and corrosion of the exposed metal surfaces.

The tarring and corrosive action of the amine-chlorinated hydrocarbon system appears to be related to certain specific metals, especially iron (also in its common alloyed forms) and copper (alone or in its alloyed forms). Aluminum on the other hand, which is known to be an 20 agent for metal induced decomposition in some cases, does not initiate the tarring and corrosion reaction in amine-stabilized systems.

In referring to "amines" in the foregoing paragraph we have used the term in its broad sense. The other organic bases specified in the Dinley patents, including cyclic compounds characterized by nitrogen in the ring, such as pyridine and morpholine, for example, are included within the meaning of this term. Among the suitable amines are 30 pyridine, di sec butylamine, diisopropylamine, diethylamine, n-butylamine, amylamines, methyl pyridines, N-methyl morpholine, triethylamine, and hexylamines.

The exact mechanism by which the amine reacts with the chlorinated hydrocarbon in the presence of the metal 40 is not completely known or understood. It may be that the amine, being a base, either forms a covalent bond with one carbon atom of the unsaturated chlorinated hydrocarbon, and the resulting fragment reacts with the metal; or, in the case of chlorinated hydrocarbons containing hydrogen, the amine may react by first removing a hydrogen to yield "ionic" fragments which in turn are reactive toward metals—the end products of such reactions being more or less complex metal organic chloro-compounds. Then again, the metal may be the initiator 45 of the set of reactions which involve the amine and the chlorinated solvent.

Regardless of what the true explanation of the phenomenon may be, serious tarring and corrosion problems 50 are encountered when an unsaturated chlorinated hydrocarbon is stabilized with an amine and the product exposed to a ferrous or cuprous metal, particularly when the hydrocarbon is hot and bone-dry.

60 It is accordingly an object of this invention to provide a method for overcoming the foregoing disadvantages, thereby providing an improved tarring and corrosion inhibiting stabilizer composition for the lower boiling un-

saturated chlorinated hydrocarbons. Other objects and advantages of this invention will further appear hereinafter.

In accordance with this invention, the tarring and corrosive action of the organic amine in the presence of certain metals and the chlorinated hydrocarbon is inhibited by incorporating into the mixture a small amount of an oxygen-containing compound. The oxygen compound does not interfere with the stabilizing action of the amine, or its ability to act as an alkaline material or to act as a reducing agent. The oxygen-containing compounds utilized in accordance with the method of this invention are epoxy compounds. It appears that these oxygen compounds may act to retard or interfere with the tarring and corrosive activity of the amine-chlorinated hydrocarbon system either by blocking the tarring and corrosive activity of the amine-stabilized system or by forming a protective layer over the surface of the metal. In the former case the amount of oxygen compound required to control the action of the amine would be related to the amount of amine used, while in the latter case the amount of oxygen compound required would be related to the surface area of the metal exposed to the solvent and amine. The amount of oxygen compound required seems to be related to the amount of amine.

It has been found that metal tarring and corrosion which occurs in the amine-chlorinated solvent-metal system containing only the usual stabilizing amount of amine can be reduced by using much larger quantities of amine. This larger quantity of amine may be of the order of ten times the usual stabilizing amount. It is believed that these very large quantities of amine may form a protective coating on the metal surface, thus interfering with the reaction between the amine, the chlorinated solvent and the metal. This method of controlling the tarring and corrosion of the metal is not desirable because the normal gradual reduction in amine content during use will bring the amine concentration into the range where the tarring and corrosion of the metal will rapidly increase and the difficulties described above be encountered; moreover, the use of such large amounts of amine greatly increase solvent stabilization costs and may introduce highly objectionable odors into solvent.

The epoxy compounds which are useful in accordance with the method of this invention are organic compounds having the linkage



The following epoxy compounds are illustrative of compounds useful in this invention:

(1) Epichlorohydrin



(2) Butylene oxides



(3) Cyclohexene oxide



In accordance with this invention the crude unsaturated chlorinated hydrocarbon, prior to the refining operation, may be combined with a stabilizing proportion of amine. The stabilized product is combined with an inhibitive proportion of an epoxy compound. The epoxy compound is chosen so that it has a boiling point slightly higher than that of the amine-stabilized chlorinated hydrocarbon being refined. This results in higher concentrations of the epoxy compound in the liquid phase than in the vapor phase and in an inhibition of the metal tarring and corrosion which would otherwise occur in the hot anhydrous amine-stabilized solvent in the bottom of the still during distillation. The amine, and not the epoxide, stabilizes the chlorinated solvent.

Unsaturated chlorinated hydrocarbons such as trichlorethylene and perchlorethylene are widely used as degreasing solvents, cleaners and the like. For example, ferrous metals are degreased commercially by subjecting them to the liquid and vapor phases of chlorinated hydrocarbons. When the chlorinated hydrocarbon is hot, dry and amine-stabilized, there is some danger of tarring and corrosion of the degreasing apparatus or of metal immersed in the liquid. Accordingly, it is commercially advantageous to provide a chlorinated hydrocarbon solvent which contains both an amine and an oxygen compound in accordance with the method of this invention.

It is well known in the art that the proportions of amine stabilizers may vary from trace values (such as .01% by weight or less) to as high as 1.0% by weight, based on the weight of the chlorinated hydrocarbon. However, a range of the order of about .02-.20% by weight represents the proportions considered commercially preferable in most amine-stabilized chlorinated hydrocarbons. Amine stabilizers have been well known and extensively used, and different amines have been used in various proportions for individual chlorinated hydrocarbons. The art is well aware of the proper concentration of each specific amine stabilizer in each specific chlorinated hydrocarbon, and such concentrations are conveniently referred to as "stabilizing amounts" and are so defined herein.

The concentration of the oxygen-containing compound may be varied from about .01% by weight to about 5% by weight, but a range of about .01-1.0% by weight is preferred. Such concentrations are referred to as "inhibitive amounts," and are so defined herein. Preferably the quantity of oxygen-containing compound is about 1-5 times the quantity of amine stabilizer.

The corrosion and tarring inhibiting effects of the addition of the oxygen compounds of the present invention may readily be shown by simple tests. These tests involve periods of refluxing of solvent samples with weighed ferrous or cuprous strips partially immersed in the liquid phase of the solvent. A group of tests is run to compare the effects of various systems. A typical group would consist of the following samples:

- (a) Solvent and metal strip
- (b) Amine-stabilized solvent and metal strip
- (c) Amine-stabilized solvent, oxygen compound and metal strip
- (d) Solvent, oxygen compound and metal strip.

The typical results of each of these tests may be summarized as follows:

Test (a): The metal strip was in good condition after reflux, showing very little or no corrosion or tarring.

The solvent showed definite signs of breakdown as would be expected.

Test (b): The metal strip showed considerable tarring and corrosion after reflux. While the degree of tarring and corrosion varied somewhat with different amines the characteristic tarring and corrosion by amine-stabilized solvent was always apparent. The solvent showed varying degrees of breakdown from none to considerable, depending on the length of the test and the amine chosen.

Test (c): The metal strip showed dramatically reduced tarring and corrosion. The solvent showed varying degrees of breakdown from almost none to considerable, depending on the length of the test and the amine chosen.

Test (d): The metal strip was in good condition after reflux, showing very little or no corrosion or tarring. The solvents showed definite signs of breakdown.

The results of reflux tests of the type described with various combinations of stabilizers and inhibitors are given in Tables IA and IB.

TABLE IA  
Reflux Tests With Trichlorethylene

| Metal  | Amine                    | Oxirane              | Corrision           | Tarring          |
|--------|--------------------------|----------------------|---------------------|------------------|
| Steel  | None                     | None                 | None                | None             |
| Copper | do                       | do                   | do                  | do               |
| Steel  | Triethylamine 0.01%      | do                   | Very bad.           | Do.              |
| Copper | do                       | do                   | do                  | Very heavy.      |
| Steel  | Diisopropylamine 0.0125% | do                   | Bad                 | Heavy.           |
| Copper | do                       | do                   | do                  | Do.              |
| Steel  | Triethylamine 0.01%      | Butylene oxide 0.05% | Slight              | Slight.          |
| Copper | do                       | do                   | do                  | do               |
| Steel  | do                       | do                   | Very slight.        | Do.              |
| Copper | do                       | do                   | do                  | Almost none.     |
| Steel  | do                       | do                   | do                  | Do.              |
| Copper | do                       | do                   | do                  | Light to medium. |
| Steel  | Diisopropylamine 0.0125% | Pentene oxide 0.05%  | Slight to moderate. | Light to medium. |
| Copper | do                       | do                   | do                  | Do.              |
| Steel  | Triethylamine 0.02%      | Butylene oxide 0.10% | Very slight.        | Very slight.     |
| Copper | do                       | do                   | Slight.             | Slight.          |

TABLE IB  
Reflux Tests With Perchlorethylene

| Metal  | Amine                     | Oxirane | Corrosion    | Tarring      |
|--------|---------------------------|---------|--------------|--------------|
| Steel  | None                      | None    | None         | None.        |
| Copper | do                        | do      | do           | Do.          |
| Steel  | N-methyl morpholine 0.01% | do      | Very bad.    | Very heavy.  |
| Copper | do                        | do      | Bad          | Heavy.       |
| Steel  | do                        | do      | Slight.      | Slight.      |
| Copper | do                        | do      | do           | Do.          |
| Steel  | do                        | do      | Very slight. | Very slight. |
| Copper | do                        | do      | do           | Slight.      |
| Steel  | do                        | do      | do           | Do.          |
| Copper | do                        | do      | do           | Do.          |
| Steel  | do                        | do      | do           | Do.          |
| Copper | do                        | do      | do           | Do.          |
| Steel  | do                        | do      | do           | Do.          |
| Copper | do                        | do      | do           | Do.          |
| Steel  | do                        | do      | do           | Do.          |
| Copper | do                        | do      | do           | Do.          |

In order to show the corrosive effects of amine-stabilized solvent on metal and the inhibitory effects of epoxides or substituted oxiranes, a series of reflux tests were run in which various amines were used while the metal (steel), the oxirane (epichlorhydrin), and the solvent

(trichlorethylene) were held constant. The results of these tests are shown in Table IIA:

5 TABLE IIA  
Corrosive Effect of Various Amines on Steel in Trichlorethylene and the Inhibitory Effect of an Epoxide or Oxirane (Epichlorhydrin)

|    |                           | Amine | Percent by wt. | Oxirane, percent by wt. | Hours of test | Metal loss, mgm./ft. <sup>2</sup> | Extent of tarring |
|----|---------------------------|-------|----------------|-------------------------|---------------|-----------------------------------|-------------------|
| 10 | Refined pyridine          | 0.02  | None           | 134.5                   | 1,917         | Severe.                           |                   |
|    | Do                        | 0.02  | 0.10           | 134.5                   | 178           | Slight.                           |                   |
|    | Do                        | 0.20  | None           | 134.5                   | 10,800        | Very severe.                      |                   |
|    | Do                        | 0.20  | 0.10           | 134.5                   | 58            | Very slight.                      |                   |
| 15 | Commercial pyridine.      | 0.02  | None           | 148.0                   | 1,835         | Severe.                           |                   |
|    | Do                        | 0.02  | 0.10           | 148.0                   | 47            | Very slight.                      |                   |
| 20 | Diisopropylamine          | 0.02  | None           | 165.0                   | 110           | Slight.                           |                   |
|    | Do                        | 0.02  | 0.10           | 165.0                   | 5             | None.                             |                   |
|    | Do                        | 0.20  | None           | 165.0                   | 72            | Slight.                           |                   |
|    | Do                        | 0.20  | 0.10           | 165.0                   | 10            | None.                             |                   |
|    | Amylamine                 | 0.02  | None           | 165.0                   | 1,100         | Severe.                           |                   |
|    | Do                        | 0.20  | None           | 165.0                   | 8,100         | Very severe.                      |                   |
|    | Do                        | 0.20  | 0.10           | 165.0                   | 288           | Slight.                           |                   |
| 25 | Methyl pyridine           | 0.02  | None           | 148.0                   | 1,260         | Severe.                           |                   |
|    | Do                        | 0.02  | 0.10           | 148.0                   | 43            | Very slight.                      |                   |
|    | N-methyl morpholine.      | 0.02  | None           | 62.0                    | 2,260         | Severe.                           |                   |
|    | Do                        | 0.02  | 0.10           | 157.0                   | 596           | Moderate.                         |                   |
| 30 | Refined triethylamine.    | 0.02  | None           | 124.5                   | 1,619         | Severe.                           |                   |
|    | Do                        | 0.20  | None           | 124.5                   | 787           | Moderate.                         |                   |
|    | Commercial triethylamine. | 0.02  | None           | 39.5                    | 3,800         | Very severe.                      |                   |
|    | Do                        | 0.02  | 0.10           | 156.5                   | 8             | None.                             |                   |
|    | Do                        | 0.02  | None           | 116.0                   | Heavy         | Severe.                           |                   |
|    | Do                        | 0.02  | 0.05           | 116.0                   | 0             | None.                             |                   |
|    | Do                        | 0.02  | 0.10           | 116.0                   | 0             | Do.                               |                   |
| 35 | None                      | None  | 0.10           | 165.0                   | 10            | Do.                               |                   |

A similar series of tests was run in which perchlorethylene was substituted for trichlorethylene. The results of these tests are shown in Table IIB:

40 TABLE IIB  
Corrosive Effect of Various Amines on Steel Strip in Perchlorethylene and the Inhibitory Effect of an Epoxide or Oxirane (Epichlorhydrin)

|    |                        | Amine | Percent by weight | Oxirane, percent by wt. | Hours of test | Metal loss, mgm./ft. <sup>2</sup> | Extent of tarring |
|----|------------------------|-------|-------------------|-------------------------|---------------|-----------------------------------|-------------------|
| 50 | Hexylamine             | 0.02  | None              | 136                     | 274           | Moderate.                         |                   |
|    | Do                     | 0.02  | 0.10              | 136                     | 5             | None.                             |                   |
|    | Do                     | 0.20  | None              | 136                     | 570           | Moderate.                         |                   |
|    | Diseetylamine          | 0.02  | None              | 63                      | 1,208         | Severe.                           |                   |
|    | Do                     | 0.02  | 0.10              | 63                      | 43            | None.                             |                   |
|    | Refined morpholine     | 0.02  | None              | 120                     | 253           | Slight.                           |                   |
|    | Do                     | 0.02  | 0.10              | 120                     | 0             | None.                             |                   |
|    | Do                     | 0.20  | None              | 120                     | 605           | Severe.                           |                   |
| 55 | Commercial morpholine. | 0.02  | None              | 63                      | 1,185         | Do.                               |                   |
|    | N-methyl morpholine.   | 0.02  | None              | 72                      | 585           | Do.                               |                   |
|    | Do                     | 0.10  | None              | 72                      | 668           | Do.                               |                   |
|    | Do                     | 0.02  | 0.05              | 87                      | 0             | None.                             |                   |
| 60 | Pyridine               | 0.02  | None              | 120                     | 122           | Slight.                           |                   |
|    | Do                     | 0.02  | 0.05              | 72                      | None          | None.                             |                   |
|    | Do                     | 0.02  | 0.10              | 120                     | 5             | Do.                               |                   |
|    | Do                     | 0.20  | None              | 120                     | 348           | Moderate.                         |                   |
|    | Do                     | 0.20  | 0.10              | 120                     | 9             | None.                             |                   |
|    | Triethylamine          | 0.02  | None              | 16                      | Heavy         | Severe.                           |                   |
|    | Do                     | 0.02  | 0.05              | 96                      | None          | None.                             |                   |
|    | Do                     | 0.02  | 0.05              | 144                     | do            | Do.                               |                   |
|    | Do                     | 0.02  | 0.10              | 144                     | None          | Do.                               |                   |
|    | Do                     | 0.02  | 0.05              | 87                      | do            | Do.                               |                   |
| 65 | None                   | None  | 0.10              | 87                      | do            | Do.                               |                   |

When a crude chlorinated solvent is refined by distillation the vapors are immediately cooled on arrival at the condenser. This results in a practical absence of solvent-amine tarring and corrosion at the condenser. The tarring and corrosion is concentrated in the reboiler where the dry amine-stabilized solvent is heated to boiling. The result is that good results in prevention of tarring and corrosion in the reboiler are obtained with

the use of an epoxy compound boiling slightly higher than the amine-stabilized solvent.

When a chlorinated solvent is used in degreasing, particularly vapor degreasing, the amine-stabilized solvent is heated in the boil sump. The amine-stabilized solvent vapors are, however, used to heat the work going into the degreaser. This results in the work being in contact with hot dry liquid amine-stabilized solvent. In this case best results are obtained if a combination of inhibitors is used. One inhibitor may be chosen to boil slightly below the amine stabilized solvent while the other may be chosen to boil slightly above the amine stabilized solvent.

The following examples will serve to show the best mode of accomplishing the above objectives:

## EXAMPLE 1

|                   | Percent |
|-------------------|---------|
| Trichlorethylene: |         |
| Triethylamine     | 0.01    |
| Butylene oxide    | 0.05    |

## EXAMPLE 2

| Trichlorethylene: |      |
|-------------------|------|
| Triethylamine     | 0.01 |
| Butylene oxide    | 0.03 |
| Epichlorhydrin    | 0.02 |

## EXAMPLE 3

| Trichlorethylene: |        |
|-------------------|--------|
| Diisopropylamine  | 0.0125 |
| Pentene oxide     | 0.05   |

## EXAMPLE 4

| Perchlorethylene:       |      |
|-------------------------|------|
| N-methyl morpholine     | 0.01 |
| 1,2-diisobutylene oxide | 0.05 |

## EXAMPLE 5

| Perchlorethylene:   |      |
|---------------------|------|
| N-methyl morpholine | 0.01 |
| Epichlorhydrin      | 0.02 |
| Cyclohexene oxide   | 0.03 |

## EXAMPLE 6

| Perchlorethylene:   |      |
|---------------------|------|
| N-methyl morpholine | 0.01 |
| Epichlorhydrin      | 0.03 |

In this specification and claims the terms "epoxy" and "oxirane" are used synonymously. The tests clearly show that the amine stabilizes the solvent while the epoxy compound does not. They also show that the presence of the amine results in tarring and corrosion while the addition of the epoxy compound to the amine-stabilized solvent results in a dramatic reduction of tarring and corrosion. The solvent alone or with the epoxy compound does not appreciably cause metal corrosion or tarring under the conditions of these tests. The epoxy compound does not stabilize the solvent, it has the unexpected result of inhibiting tarring and corrosion in an amine stabilized system.

Having thus described our invention, we claim:

1. In a process wherein a metal selected from the class consisting of ferrous and cuprous metals is exposed to a hot, dry, unsaturated low molecular weight chlorinated hydrocarbon selected from the class consisting of trichloroethylene and perchlorethylene, and containing a stabilizing amount of a volatile organic nitrogen compound selected from the group consisting of aliphatic amines and heterocyclic nitrogen bases, said nitrogen compound stabilized chlorinated hydrocarbon normally causing tarring and corrosion of said metal, the improvement which comprises incorporating into said nitrogen compound stabilized chlorinated hydrocarbon about .01-5% by weight of an inhibitor for said metal tarring and corrosion comprising a substituted oxirane selected from the class consisting of epichlorhydrin, butylene oxide, pentene oxide, cyclohexene oxide and 1,2-diisobutylene oxide.
2. The process of claim 1 wherein said substituted oxirane has a boiling point higher than that of said stabilized solvent.

iran has a boiling point higher than that of said stabilized solvent.

3. In a method of refining a crude volatile low molecular weight chlorinated unsaturated hydrocarbon solvent selected from the class consisting of trichloroethylene and perchlorethylene in the presence of a metal selected from the class consisting of ferrous and cuprous metals, said solvent having incorporated therein a stabilizing amount of a volatile organic nitrogen compound selected from the group consisting of aliphatic amines and heterocyclic nitrogen bases, said nitrogen compound stabilized solvent normally causing tarring and corrosion of said metal, the improvement which comprises incorporating into said nitrogen compound stabilized chlorinated hydrocarbon about .01-5% by weight of an inhibitor for said metal tarring and corrosion comprising a substituted oxirane selected from the class consisting of epichlorhydrin, butylene oxide, pentene oxide, cyclohexene oxide and 1,2-diisobutylene oxide, wherein said substituted oxirane has a boiling point higher than that of the nitrogen compound stabilized chlorinated hydrocarbon.

4. In a process of degreasing metal surfaces selected from the class consisting of ferrous and cuprous metals with a hot, volatile, unsaturated chlorinated hydrocarbon selected from the class consisting of trichloroethylene and perchlorethylene, and containing a stabilizing amount of a volatile organic nitrogen compound selected from the group consisting of aliphatic amines and heterocyclic nitrogen bases, said nitrogen compound stabilized chlorinated hydrocarbon normally causing tarring and corrosion of said metal, the improvement which comprises incorporating into said nitrogen compound stabilized chlorinated hydrocarbon about .01-5% by weight of an inhibitor for said metal tarring and corrosion comprising a substituted oxirane selected from the class consisting of epichlorhydrin, butylene oxide, pentene oxide, cyclohexene oxide and 1,2-diisobutylene oxide.

5. In a process of degreasing metal surfaces selected from the class consisting of ferrous and cuprous metals with a hot, volatile, unsaturated chlorinated hydrocarbon selected from the group consisting of trichloroethylene and perchlorethylene, and containing a stabilizing amount of a volatile organic nitrogen compound selected from the group consisting of aliphatic amines and heterocyclic nitrogen bases, said nitrogen compound stabilized chlorinated hydrocarbon normally causing tarring and corrosion of said metal, the improvement which comprises incorporating into said nitrogen compound stabilized chlorinated hydrocarbon about .01-5% by weight of a combination of at least two inhibitors for said metal tarring and corrosion, each of said inhibitors comprising a substituted oxirane selected from the class consisting of epichlorhydrin, butylene oxide, pentene oxide, cyclohexene oxide and 1,2-diisobutylene oxide, wherein at least one of said inhibitors has a boiling point higher than that of said nitrogen compound stabilized solvent, and at least one of said inhibitors has a boiling point lower than that of said nitrogen compound stabilized solvent.

6. The process of claim 5, wherein the substituted oxiranes are butylene oxide and epichlorhydrin.

7. The process of claim 5, wherein the substituted oxiranes are butylene oxide and cyclohexene oxide.

8. The process of claim 5, wherein the substituted oxiranes are pentene oxide and epichlorhydrin.

9. The process of claim 5, wherein the substituted oxiranes are pentene oxide and cyclohexene oxide.

10. The process of claim 5, wherein the substituted oxiranes are pentene oxide and 1,2-diisobutylene oxide.

11. The process of claim 5, wherein the substituted oxiranes are epichlorhydrin and cyclohexene oxide.

12. The process of claim 5, wherein the substituted oxiranes are epichlorhydrin and 1,2-diisobutylene oxide.

13. In a process of degreasing objects having metal surfaces selected from the class consisting of ferrous and cuprous with a hot, volatile, unsaturated chlorinated hy-

drocarbon, said chlorinated hydrocarbon being selected from the group consisting of trichlorethylene and perchlorethylene, said chlorinated hydrocarbon having incorporated therein a stabilizing amount of a volatile organic nitrogen base selected from the group consisting of pyridine, di sec butylamine, diisopropylamine, diethyl amine, n-butylamine, amyamine, methyl pyridine, N-methyl morpholine, triethylamine and hexylamine, said nitrogen compound stabilized solvent normally causing tarring and corrosion of said metal surfaces, the improvement which comprises incorporating into said nitrogen compound stabilized chlorinated hydrocarbon about .01-5% by weight of an inhibitor for said metal tarring and corrosion comprising a substituted oxirane selected from the class consisting of epichlorhydrin, butylene oxide, pentene oxide, cyclohexene oxide and 1,2-diisobutylene oxide, wherein said substituted oxirane has a boiling point higher than

that of the nitrogen compound stabilized chlorinated hydrocarbon.

14. The process of claim 13 wherein said substituted oxirane is epichlorhydrin.

References Cited in the file of this patent

UNITED STATES PATENTS

|    |           |                 |               |
|----|-----------|-----------------|---------------|
| 10 | 2,043,257 | Missbach        | June 9, 1936  |
|    | 2,364,588 | Morris et al.   | Dec. 5, 1944  |
|    | 2,371,644 | Petering et al. | Mar. 20, 1945 |
|    | 2,371,645 | Aitchison       | Mar. 20, 1945 |
|    | 2,371,646 | Petering et al. | Mar. 20, 1945 |
| 15 | 2,797,250 | Copelin         | June 25, 1957 |
|    | 2,947,792 | Skeeters        | Aug. 2, 1960  |
|    | 2,973,392 | Graham          | Feb. 28, 1961 |
|    | 2,978,518 | Daras           | Apr. 4, 1961  |
|    | 2,981,760 | Ferri et al.    | Apr. 25, 1961 |

UNITED STATES PATENT OFFICE  
CERTIFICATE OF CORRECTION

Patent No. 3,133,885

May 19, 1964

Wilbur H. Petering et al.

It is hereby certified that error appears in the above numbered patent requiring correction and that the said Letters Patent should read as corrected below.

Column 3, line 61, for "compounds" read -- compounds --; column 4, line 49, for "conveniently" read -- conventionally --; column 6, TABLE IIA, line 3 of the heading thereof, for "Oxriane", in italics, read -- Oxirane --, in italics; column 7, line 71, for "compris-" read -- comprising --; column 8, line 75, after "cuprous" insert -- metals --.

Signed and sealed this 20th day of October 1964.

(SEAL)  
Attest:

ERNEST W. SWIDER  
Attesting Officer

EDWARD J. BRENNER  
Commissioner of Patents